

Jan. 10, 1950

M. P. MONTERO

2,494,351

FIBER-REINFORCED BOWLING PIN

Filed Dec. 17, 1947



Fig. 1

Fig. 2



Fig. 4

INVENTOR.  
MODESTO P. MONTERO  
BY *Edward M. Morris*  
ATTORNEY.

## UNITED STATES PATENT OFFICE

2,494,351

## FIBER-REINFORCED BOWLING PIN

Modesto P. Montero, Newark, N. J.

Application December 17, 1947, Serial No. 792,145

1 Claim. (Cl. 273—82)

1

This invention relates to new and useful improvements in bowling pins.

Heretofore attempts have been made to construct bowling pins more durable than the usual wooden bowling pins. However, these prior attempts did not meet with material commercial success for numerous reasons. If the materials from which they were constructed were more durable, the sound of the pins when struck with the bowling ball in the playing of a match was not satisfactory. If the sound was satisfactory then the material did not possess all desirable physical properties of strength, durability, etc.

This invention proposes a new and improved bowling pin and a method for its construction which will have a satisfactory sound when struck by the bowling ball during play, and which will be more durable than pins heretofore used.

The invention proposes to accomplish the main objects stated in the prior paragraph by making use of a strip of vulcanized fibre bonded around the central bellied body portion of the pin. A certain substance is proposed for bonding the vulcanized fibre strip in position to eliminate air spaces and pockets which otherwise would give the pin a hollow sound, or a split sound, when struck by a bowling ball, which sounds are highly objectionable to master players.

Another object of the invention is the construction of a bowling pin as described which is simple and durable and which may be manufactured and sold at a reasonable cost.

For further comprehension of the invention, and of the objects and advantages thereof, reference will be had to the following description and accompanying drawing, and to the appended claim in which the various novel features of the invention are more particularly set forth.

In the accompanying drawing forming a material part of this disclosure:

Fig. 1 is a front elevational view of the body portion of a bowling pin formed with a circumferential groove required for constructing the bowling pin in accordance with this invention.

Fig. 2 is a fragmentary perspective view of a strip of vulcanized fibre used in the construction of the new bowling pin.

Fig. 3 is a fragmentary enlarged central vertical sectional view of an unfinished bowling pin constructed from the body portion illustrated in Fig. 1 upon which the vulcanized fibre strip, illustrated in Fig. 2, has been applied.

Fig. 4 is a sectional view similar to Fig. 3 but illustrating the finished bowling pin.

The construction of the new and improved

2

bowling pin may be best understood by studying the method by which it is constructed. A wooden bowling pin body portion 10 of standard form has a circumferential groove 11 formed in the portion which is normally the central bellied portion of the bowling pin. The bowling pin body portion 10 may be a new bowling pin body portion or may be formed from an old bowling pin which is to be refinished. The circumferential groove 11 has a cylindrical base wall 12 and top and bottom shoulders 13 and 14, respectively. The dot and dash lines 15 in Fig. 1 indicate the normal shape of the central bellied portion of the bowling pin. If the bowling pin body portion 10 is made from an old bowling pin that is being refinished, then the bellied central portion 15 is turned down. If the bowling pin body portion 10 is a new one it may be made from a smaller size of wood stock than the usual all wooden bowling pin and turned down into the required shape.

Fig. 2 illustrates a strip of vulcanized fibre 16. Any of the well known vulcanized fibre strip materials now on the market may be used. This material has a high impact strength, is arc resistant, and is formable and machinable. It is proposed that the strip 16 be wound around the circumferential groove 11. First the end portion of the strip 16 should be beveled, preferably by sanding. The line AB divides off a section of the end portion of said strip 16. The bevel should be formed from the line AB to the left hand end of the strip 16. Then the vulcanized fibre strip 16 is softened, preferably with steam. A coating of a specially prepared animal glue is applied to the strip 16 and it is wound around and around in the groove 11 to the shape illustrated in Fig. 3. The strip 16 must be long enough so that it can be wound around a number of times to a diameter equal to or slightly greater than the normal large diameter of the central bellied body portion of the bowling pin.

It is very important that the vulcanized fibre strip 16 be applied in position in a manner so that there are no air spaces or air pockets between the wound layers thereof, because such spaces or pockets will interfere with the sound of the pin when struck by a bowling ball. Air spaces and pockets will give the pin a hollow or split sound. I have discovered that if ordinary animal glue is used it is virtually impossible to avoid the existence of spaces or air pockets between the wound layers of the vulcanized fibre strip. I have furthermore discovered that all spaces and air pockets can be eliminated if the wound on vulcanized fibre strip is caused to

swell so as to close all spaces and air pockets and is furthermore caused to become "set" in its enlarged condition. I accomplish this by adding an alkali to the glue to cause the vulcanized fibre strip to swell, and by adding formaldehyde to the glue to "set" the swollen vulcanized fibre strip and prevent it from contracting when the glue dries.

In order to better understand the invention one formula of glue will be given. Take 9 lbs. of dry animal glue and about 1 lb. of formaldehyde and add the necessary water and boil to produce a glue of proper consistency. Then add an alkali, like carbonate of soda to raise the pH of the prepared glue to a pH of from 8 to 10. While this is the particular formula I have used successfully it should be understood that any specially prepared animal glue would be satisfactory provided it is prepared with formaldehyde and with the addition of any alkaline substance which would produce a glue having a pH of from 8 to 10. A glue with an alkaline reaction has a chemical action which will soften the vulcanized fibre strip 16 causing the fibre strip 16 to swell, and it is this swelling which presses out and closes all spaces and pockets. The formaldehyde enters the enlarged pores of the swollen vulcanized fibre strip and then solidifies and prevents the swollen strip from contracting.

Preferably a clamp (not illustrated on the drawing) is engaged about the center of the wound strip 16 on the pin body portion 10, as illustrated in Fig. 3, and the special glue is permitted to dry and harden to bond the strip 16 in its wound condition on the bowling pin body portion. When suitably dried and bonded the projecting portions of the wound vulcanized fibre strip 16, are machined down into the proper central bellied body portion shape. The bowling pin is then finished with a protective coating 18 of paint, or other suitable protective or covering material.

It is also advisable that the bowling pin be provided with a bottom protective bushing 20 of vulcanized fibre material having a bottom opening 21 to reinforce and to protect the bottom of the pin and prevent its rapid wearing out during use.

An important feature of the new bowling pin resides in the fact that the vulcanized fibre strip central bellied body portion of the pin is excep-

tionally strong and capable of withstanding severe impacts. The bowling pin is therefore strong and durable. Moreover, these bowling pins have a very desirable sound when hit by a 5 bowling ball during a game, a sound which is not objectionable to the best masters in the game. When a bowling pin has a poor sound, or when it sounds split or hollow, and a master obtains a bad shot he is apt to blame it on the bowling pins. However these new bowling pins are satisfactory in all respects.

While I have illustrated and described the preferred embodiment of my invention, it is to be understood that I do not limit myself to the precise construction herein disclosed and the right is reserved to all changes and modifications coming within the scope of the invention as defined in the appended claim.

Having thus described my invention, what I 20 claim as new and desire to secure by United States Letters Patent is:

The combination with a bowling pin having a wound strip of vulcanized fibre in its body portion, of material bonding the turns of said vulcanized fibre together, said material comprising an animal glue containing formaldehyde and an alkali, said alkali giving said animal glue a pH of from 8 to 10 so that said alkali is able to swell said wound strip to close spaces and air 25 pockets in the turns of said wound strip, and said formaldehyde acting to "set" said swollen strip to prevent it from contracting as said glue dries so that no new spaces and air pockets are formed.

35

MÓDESTO P. MONTERO.

## REFERENCES CITED

The following references are of record in the 40 file of this patent:

## UNITED STATES PATENTS

| Number     | Name      | Date           |
|------------|-----------|----------------|
| Re. 19,128 | Drew      | Apr. 3, 1934   |
| 846,164    | Tector    | Mar. 5, 1907   |
| 925,128    | McGuire   | June 15, 1909  |
| 1,110,487  | Hillerich | Sept. 15, 1914 |
| 1,227,248  | Crane     | May 22, 1917   |
| 1,429,427  | Herstein  | Sept. 19, 1922 |
| 2,105,045  | Kraft     | Jan. 11, 1938  |
| 2,379,006  | Johnson   | June 26, 1945  |